

Patented Mar. 18, 1924.

1,487,521

# UNITED STATES PATENT OFFICE.

PAUL ANDREU AND RENÉ PAQUET, OF PARIS, FRANCE.

## FIXATION OF NITROGEN BY MEANS OF TITANIUM AND ITS TRANSFORMATION INTO INDUSTRIAL PRODUCTS.

No Drawing.

Application filed January 13, 1922. Serial No. 529,028.

To all whom it may concern:

Be it known that we, PAUL ANDREU and RENÉ PAQUET, citizens of the French Republic, residing at Paris, Department of the Seine, in France, have invented certain new and useful Improvements in the Fixation of Nitrogen by Means of Titanium and Its Transformation into Industrial Products, of which the following is a specification.

The present invention has for its object the fixation of nitrogen by means of titanium and its transformation into industrial products, such as cyanides, ammonia, etc., together with, if desired, the extraction of the titanium contained in minerals such as titanium irons, rutiles, anatase, etc.

If the extraction of the titanium or its salts be desired, the following process is employed:

The titanium ore is mixed with charcoal and a salt of a metal, alkali, alkaline earth or the like (for example sodium carbonate). The whole is then reduced to powder. The quantities to be used are varied in accordance with the analysis of the ore. The following mixture is given by way of example:

|                                          | kgs.  |
|------------------------------------------|-------|
| Titanium iron ore containing 40% $TiO_2$ | 1,000 |
| Sodium carbonate                         | 750   |
| Charcoal                                 | 1,000 |

This mixture should be heated in an atmosphere of nitrogen to a temperature not exceeding  $1,850^{\circ}$  C. The mixture will absorb the nitrogen and will give nitrides and carbides, etc., which will then be subjected to the action of steam at a temperature not exceeding  $1,800^{\circ}$  C., giving off ammonia, hydrocyanic acid, etc. These various products will be collected by means of suitable washing or condensing apparatus.

The mass, having been subjected to the action of steam will contain a large part of the metals in the form of oxides and the titanium in the form of titanate which can be extracted by washing with water, acids, and bases. The washing with water dissolves the titanate and thereby separates the titanium from the iron. The titanium solution is then precipitated by hydrolysis by the action of acids or bases.

After washing, filtering, drying and calcining at a high temperature an anhydrous

product composed of titanium oxide will be obtained.

The above description is given by way of example only and the details can be modified without departing from the scope of the invention, which consists in fixing the nitrogen in the presence of or by means of titanium and forming therefrom industrial products with the possibility of separating the titanium or its salts. It will be understood the fixation of the nitrogen only may be effected by employing modifications of the above process such, for instance, as nitrogenizing a mixture of the ore and charcoal only, then subjecting it to the action of steam and recovering the volatile products (in which case the solid residue can be employed over again) lixiviation may follow the nitrogenizing thus obtaining directly cyanides, sulpho-cyanides, ferro-cyanides, etc.

We claim—

1. A process of producing titanium oxide with simultaneous recovery of nitrogen compounds which comprises mixing a titanium containing ore, with about an equal weight of carbonaceous material and amount of an alkali corresponding to about three-fourths said weight of sodium carbonate, subjecting the mixture to an atmosphere containing free nitrogen at a temperature near  $1850^{\circ}$  C., and thereafter subjecting the resulting product to action of steam at near  $1800^{\circ}$  C., whereby nitrogen compounds are evolved, leaching the solid product with water whereby the soluble titanium compounds are separated from iron and other insoluble materials, subjecting the resulting solution to hydrolytic dissociation and calcining the product.

2. A process of producing titanium oxide with simultaneous recovery of nitrogen compounds which comprises mixing one hundred parts of titanium ore containing about 40%  $TiO_2$ , one hundred parts of carbon and seventy-five parts of  $Na_2CO_3$ , subjecting the mixture to an atmosphere containing free nitrogen at a temperature near  $1850^{\circ}$  C., and thereafter subjecting the resulting product to action of steam at near  $1800^{\circ}$  C., whereby nitrogen compounds are evolved, leaching the solid product with water whereby the soluble titanium compounds are separated from iron and other insoluble materials, subjecting the result-

ing solution to hydrolytic dissociation and calcining the product.

3. A process which comprises heating to a high temperature, in an atmosphere of nitrogen, a mixture containing titanium ore, alkali and a carbonaceous material, the proportion of alkali to titanium ore corre-

sponding to about 75 parts by weight of sodium carbonate to each 40 parts of  $TiO_2$  in the said ore.

In testimony whereof we hereunto affix our signatures.

PAUL ANDREU.  
RENÉ PAQUET.